

Dec. 24, 1940.

R. K. HOPKINS

2,226,403

MANUFACTURE OF VENEERED ARTICLES

Filed July 23, 1938



FIG. 1



FIG. 2



FIG. 3



FIG. 4

INVENTOR  
ROBERT K. HOPKINS  
BY  
*Virgil F. Davis*  
ATTORNEY

## UNITED STATES PATENT OFFICE

2,226,403

## MANUFACTURE OF VENEERED ARTICLES

Robert K. Hopkins, New York, N. Y.

Application July 23, 1938, Serial No. 220,853

4 Claims. (Cl. 80—60)

This invention relates to the manufacture of coated or veneered articles, more particularly the invention relates to the conversion of thick, coated or veneered, metal bodies into thinner worked bodies.

In my prior Patents, No. 2,151,194 of March 28, 1939, and No. 2,191,469 of February 27, 1940, are disclosed new methods for making coated articles. The new methods briefly, include the deposition 10 of fusing metal on the surface of a base metal under a blanket of flux of substantially non-gassing character and of a sufficient thickness to protect the metal depositing operation from the atmosphere. The fusing metal is deposited by 15 means of electric current discharge beneath the flux blanket through a gap, or gaps, between one or more electrodes and the base metal. The current discharge is effective to fuse metal of the electrode, or electrodes, and a depth of the metal 20 of the base so that these metals commingle to form the coating or veneer. The penetration into the base metal and the analysis of the metal deposited from the electrode, or electrodes, are so chosen and controlled that the final coating or 25 veneer is of the required analysis.

The coating or veneer is deposited in the form of comparatively wide bands of substantially uniform penetration and analysis. The entire surface of the base metal to be coated or veneered is 30 covered by depositing the necessary number of bands. To assure a continuous coating or veneer the bands are preferably overlapped. The thus coated or veneered base metal may be used as such but in the usual case it is rolled or otherwise 35 worked into a finished article.

The working operation converts the coated base metal into a finished article and in so doing also converts the coating or veneer material, which as deposited is substantially in the cast condition, 40 into work refined metal.

I have found that in the commercial production of coated or veneered worked articles, in accordance with the method briefly described above, and especially steel articles coated or veneered with 45 corrosion resistant alloys such as chrome steels, chrome nickel steels, etc., perfect articles are not invariably produced but imperfections are sometimes developed during the working operations. Aside from the usual imperfections such as snakes, 50 bursts, etc., which are more or less inherent in working operations, particularly roll-working operations, and which may appear on either side of the metal worked, there appear from time to time closely spaced, short, narrow checks or cracks, which are found only on the alloy side of the

article. The closely spaced checks or cracks are usually quite shallow but occasionally they extend completely through the alloy coating or veneer. Also, the checks or cracks if they appear at all, either cover the whole alloy surface of the article 5 or cover a well defined part of it; isolated checks or cracks are seldom if ever found.

The usual imperfections can, as a rule be repaired economically; this is seldom true of these unusual cracks or checks. Because of the nature 10 of the cracks or checks it is dangerous to employ articles showing them in the manufacture of apparatus, such as pressure vessels for the petroleum refining industry, that are to be subjected to extreme pressures and temperatures in the presence 15 of corrosive media.

A careful study of the problem leads to the conclusion that the closely spaced checks and cracks do 20 not result from the coating or veneering operation but are developed during the working operation. Thus, identical slabs have been coated with substantially identical veneers under the same conditions and these coated slabs rolled under non-identical conditions. Perfect plate was obtained 25 from some of these slabs and plate of varying degrees of imperfection attained from others of the slabs.

It is the primary object of this invention to 30 provide a novel method for working metal bodies having a coating of veneer metal of different composition integrally united to them throughout, in which the metal bodies are work deformed into the final articles without producing closely spaced checks and cracks in the surface of the veneer 35 metal.

It is a further object of this invention to provide a method for heat treating metal bodies having a coating of veneer metal of different composition integrally united to them throughout, by 40 means of which the full thickness of the metal bodies are brought to such a degree of plasticity that they can be work deformed into final articles without producing closely spaced checks and cracks in the surface of the veneer metal. 45

The further objects and advantages of the invention will be better appreciated from a consideration of the following detailed description of present preferred modes for carrying it out in practice, taken with the accompanying drawing, 50 in which:

Fig. 1 is a schematic view partly in section illustrating the manner in which the coating or veneer is applied to the base metal,

Figs. 2 and 3 are schematic views, in section, il- 55

Iustrating roll working of coated or veneered bodies, and

Fig. 4 is a fragmentary view on a larger scale of the subject matter of Fig. 2.

5 The invention is of general application and may be used in the working of coated or veneered metal bodies of a wide range of compositions, however, since steel, either plain carbon steel or carbon steel that includes low percentages of alloying elements such as chromium, manganese, molybdenum, nickel, etc., is the most common of the metals used as base metal for coated or veneered articles, and the corrosion resisting alloys such as chrome steel, chrome nickel steel, etc., 10 are the most common metals used to form the coating or veneer, the invention will be described in connection with the manufacture of coated or veneered articles that include a steel base and a corrosion resisting coating or veneer. Also, while 15 a wide variety of coated or veneered articles may be manufactured by various working operations the invention will be described in connection with roll working for the manufacture of flat articles such as plates, sheets, etc.

20 25 The workpiece employed in the manufacture of the flat article just mentioned is preferably a thick steel slab coated with a correspondingly thick veneer of the chosen analysis, thus, the slab may range in thickness from six inches, or less, to twenty-four inches or more, and the coating may range from one-half an inch, or less, to several inches or more depending on the thickness of the final desired article and the reduction desired.

30 35 To form the workpiece, a steel slab 10 is positioned beneath a suitable welding head 11. Welding head 11 may be of any preferred type and construction but should include arrangements for supplying electric current at controllable voltages and amperages, and arrangements for automatically feeding, either independently or in parallel, electrodes 12 (two being shown but a lesser or greater number may be employed) to maintain electrical discharge of predetermined 40 characteristics. Head 11 may include a current generator or may be provided with current connections to an outside source. Current is supplied to work 10 by cable 15 and to contact devices 14, through which electrodes 12 pass, by cable 13.

45 50 55 60 65 70 75

Electrode or electrodes 12 may be solid or hollow, of any preferred cross section, and may include all of the constituents necessary to form the desired alloy coating or veneer, when the metal fused from the electrodes and the work intermingle, or they may include only some of the constituents and the remainder supplied from an external source such as flux blanket 16, a metal bar, etc. At present, I prefer to employ a plurality of electrodes that includes one or more hollow electrodes and supply the remainder of the required constituents through the hollow electrodes. When the chosen coating or veneer is chrome steel, the hollow electrode is preferably of mild steel and the required chromium is supplied as ferro-chrome through the hollow electrode; when the chosen coating is chrome-nickel steel the chromium is supplied as ferro-chrome as before and the nickel is supplied as powder, pellets, etc. With some alloys, as for instance chrome-nickel steel, it is sometimes preferable to make one or more of the hollow electrodes and/or one or more of the other electrodes of a metal other than steel, as for instance nickel as all of

the iron required, may sometimes be supplied by the base and the remainder of the electrodes.

The electrodes 12 are fed until they almost touch work 10 and arc starters placed between them and base 10. The surface of work 10 to be 5 coated or veneered is then covered with a blanket of flux 16 of sufficient depth to submerge the coating or veneering operation and to protect it as well as the fused metal from the atmosphere. Flux blanket 16 may be from an inch to six 10 inches, or more, deep and is confined at the area to be coated by dams 17.

The flux should be such that it will not liberate deleterious gas, either as to quantity or kind, and will not add substantial quantities of undesirable ingredients to or remove substantial quantities of desirable ingredients from the molten metal but will flux out impurities. A wide variety of fluxes may be used satisfactorily. Silicates, simple or compound or a mixture of these, aluminates, titanates, and the like, are satisfactory. The flux may be prefused or it may be made up of dried or calcined components. At present, silicates of the alkaline earth metals (calcium and magnesium being preferred), manganese and 25 iron are preferred fluxes.

After flux blanket 16 is laid, the electric energy circuit is closed and the operation started, the initial flow of energy will destroy the arc starters and thus provide current discharge paths between the electrodes and the surface of the work. The heat generated by the discharges will fuse a depth of metal of work 10, metal of the electrodes, and any metal passed to the gaps between the electrodes and the work with the result that an alloy pool will be formed of substantially uniform analysis that is integrally united to work 10. The heat generated will also fuse some of the flux and thus provide a molten blanket that protects the operation from the atmosphere. The electrodes are moved relative to the work to deposit the alloy in the form of a wide band 18. A band 18 of desired composition is obtained by so controlling the operation that there is continuously fused predetermined proportions of the metal of base 10 and metal from electrodes 12 and metal from other sources. The desired portion of the surface of work 10 is coated or veneered by laying a sufficient number of bands 18. In order to obtain a continuous alloy 35 40 45 50 55 60 65 70 75 coating bands 18 are overlapped somewhat.

After the coating operation is completed the coated slab is roll worked to form it into the finished article. The working operations comprise the heating of the slab to a rolling temperature 55 and the actual rolling.

While coated slab 10 is primarily a steel slab, since the greater proportion of its thickness and volume is of steel, the heating and rolling practice ordinarily employed for comparable steel 60 slabs will generally produce a finished article that shows the objectionable cracks in the surface of the coating. This results from the fact that coating 18, which while it may only be a minor proportion of the slab behaves differently than the 65 steel and requires different treatment.

If a coated slab is heated and rolled under the conditions ordinarily employed in the rolling of steel slabs, the coated slab will deform as shown in Figs. 2 and 4. Fig. 2 shows diagrammatically 70 the manner in which the surface metal of the slab is acted upon by the rollers. It is obvious from examination of this figure that if a coated slab were heated in accordance with the practice usually employed with all steel slabs the central por- 75

tion of the coated slab would not be as plastic as the remainder of the slab and would, therefore, not be susceptible to the same rate of deformation as the remainder of the slab. Because of this fact, the central portion of the slab would not be elongated solely by the decrease in thickness caused by the setting of the rollers, but partly by high tensile stresses set up in the surface of the slab and the material between the surface and the center. These high tensile stresses cause the metal of the coating to pull apart and therefore produce checks on the surface of the finished plate. This is illustrated in Fig. 4 wherein the dotted lines are intended to illustrate the crystals or grains of metal 18. The reason the coated surface checks and the carbon steel surface on the other side does not check is partly due to the dendrites existing in the as-cast alloy material and to the tenderness of this type of alloy as compared to the partially worked and inherently tougher carbon steel. Since coating metals such as chrome-steels, chrome-nickel steels do not pressure weld readily, if at all, the cracks and checks are not eliminated by subsequent passes through the rolls but as a matter of fact more of them are produced.

I have found that in order to invariably produce coated worked articles that are free, or substantially free, of the objectionable cracks and checks it is necessary that the slab be heated so it is at a substantially uniform temperature throughout its thickness and extent. The temperature should be such that the coating material will be sufficiently plastic to deform without noticeable slippage between its grains. The temperature, furthermore, should be such that the steel portion of the slab will be sufficiently plastic to deform, under the pressure applied, uniformly throughout its thickness so that a minimum of stress will be set up in the coating material.

When coated slabs heated in accordance with this invention, are rolled as in the ordinary practice, the deformation is substantially uniform throughout the slab, see Fig. 3, so that a minimum of stresses are set up that tend to crack or check the surface of the coating metal 18.

The optimum rolling temperature will vary with the analysis of the steel base 16 and the coating metal 18 and in each particular case can best be arrived at by experiment. The desired results have been obtained with coated steel slabs having a base made of plain 0.2% carbon steel and a coating made of 18-15% chrome steel by rolling at a temperature of 2300° F. Satisfactory results can generally be obtained with plain carbon steel slabs, or carbon steel slabs that include low percentages of alloying constituents such as nickel, manganese, molybdenum etc., that are coated with chromium steel or chrome-nickel steel by rolling at temperatures that initially range from 2100-2400° F. The optimum temperature will generally be substantially the lowest temperature that will give the desired plasticity to both the base and the coating. The use of higher temperatures, is not desirable. The heating to higher temperatures, while it increases the plasticity, not only increases the cost of the operation but oftentimes produces defects in the metal.

To heat the coated slab to the selected rolling temperature, so that all of the metal between its surfaces is at a substantially uniform temperature and yet deleteriously effect the metal of the slab to a minimum degree, a special technique is required. I have found that best results are obtained by initially heating the slab in a pit, fur-

nace, etc., to a surface temperature in the vicinity of the upper critical temperature of the steel base metal. The temperature of the furnace or pit is then raised until the temperature of the exposed surfaces of the slab attain a temperature that is 5 at or approaches the lower limit of the plastic range of the metals of the slab. The heat input into the furnace or pit is then controlled to maintain the surface temperature substantially constant for a period of time required to bring the 10 whole of the metal to the surface temperature. This condition will be closely approximated though never quite attained as there is of necessity a temperature gradient from the surface of the slab, the place of entrance of the heat, to the 15 metal at the center of the slab. The holding time necessary for uniform temperature throughout the slab depends on many factors such as the 20 luminescence of the heat source, the furnace or pit design, the thickness of the metals of the slab, 25 their diffusivities, their conductivities, their specific heats, densities, etc. The holding time can be calculated from formulae that are known, or at least readily available to the workers in the art and, consequently, need not be set forth here. 25 With coated slabs of the character set forth above, a holding time in the neighborhood of 15 minutes per inch of thickness of the slab will, in general, be satisfactory.

After the whole of the slab has been brought 30 to the selected temperature, at or approaching the plastic range of the metals of the slab the heat input to the furnace or pit is increased to raise the surface temperature of the slab to the predetermined rolling temperature. The heat input to the furnace or pit is then controlled to maintain the surface metal at the predetermined 35 temperature for the length of time required for the whole slab to attain a uniform temperature. The holding time is a function of the factors 40 stated above, and may be calculated from known and available formulae. With coated slabs of the character set forth above, a holding time in the neighborhood of 20 minutes per inch of thickness of the slab will give the desired results. 45 After this treatment the slab is passed to the rolls wheretofore it is worked to increase its area and reduce its thickness. The working operations convert the coating metal from metal having the characteristics of cast metal into work 50 refined metal.

As a specific example, a coated slab made up of a plain carbon steel base (0.20% carbon) 17.25 inches thick to which has been integrally united throughout, to one of the major faces thereof, 55 a coating of 18-15% chrome steel 0.75 inch thick, is charged at ordinary temperature into a furnace and heated until the surface metal attains a temperature of 1600° F. The furnace and slab may be raised in temperature together or the 60 furnace may be up to temperature when the slab is charged. The furnace employed was of the type usually employed in steel mills for heating slabs prior to rolling operations. The heat source was such as to fall within the technical 65 classification of highly luminous flame. After the 1600° F. temperature was attained, the heat input was increased to raise the surface temperature of the slab to 2000° F. It required one and one-half hours to obtain this temperature 70 increase. The heat input was then adjusted to maintain the surface temperature of the slab substantially constant for the length of time (5.5 hours) required to substantially secure this temperature throughout the depth of the slab. From 75

calculations it had been determined that a holding time of 15 minutes per inch of thickness of the slab was necessary. At the end of the 5.5 hours holding time the heat imput was again increased to raise the surface temperature to 2300° F., the temperature determined by experiment to be the satisfactory rolling temperature. This temperature increase required one hour. The heat imput was then adjusted to maintain this new surface temperature for the length of time (6 hours) necessary to substantially secure this temperature throughout the metal of the slab. It has also been determined from calculations that a holding time of 20 minutes per inch of thickness of the slab was required for this purpose. Calculations indicated that at the end of this holding time the metal at the center of the slab would attain a temperature of 2277° F. The 23° F. temperature gradient could be reduced by increasing the holding time but the added cost as well as the deleterious effects on the metals of the slab, would outweigh any advantages that could be obtained by the small increase in plasticity of the center of the slab.

25 The thus heated slab was then passed to the rolls and converted into a plate 1.5 inches thick. The plate was free from checks and cracks on its alloy surface.

I claim:

30 1. The method of manufacturing worked composite metal articles, which comprises, heating a composite workpiece, made up of a ferrous metal base to which is integrally united a protective alloy coating, to the critical range of the ferrous

35 base metal, raising the temperature of the surface metal of said workpiece to substantially the lower limit of the plastic ranges of the metals of said workpiece, maintaining said surface temperature for a time interval sufficient to raise substantially all of the metal of said workpiece to said surface temperature, further raising the temperature of the surface metal of said workpiece to a selected working temperature within the plastic ranges of the metals, maintaining said surface temperature for a time interval equivalent to substantially 20 minutes per inch of thickness of said workpiece based on a highly luminous heat source, and work deforming the said heated workpiece to form the desired worked article.

45 2. The method of manufacturing worked composite metal articles which comprises, heating a composite workpiece, made up of a ferrous metal base to which is integrally united a protective alloy coating, to the critical range of the ferrous

50

base metal, raising the temperature of the surface metal of said workpiece to substantially the lower limit of the plastic ranges of the metals of said workpiece, maintaining said surface temperature for a time interval equivalent to substantially 15 minutes per inch thickness of said workpiece based on a highly luminous heat source, further raising the temperature of the surface metal of said workpiece to the selected working temperature within the plastic ranges of the metals, maintaining said surface temperature for a time interval equivalent to substantially 20 minutes per inch of thickness of said workpiece based on a highly luminous heat source, and work deforming the said heated workpiece to form the 15 desired worked article.

3. The method of manufacturing worked composite metal articles which comprises, heating a composite workpiece, made up of a ferrous metal base to which is integrally united a corrosion resistant chromium containing alloy coating, to substantially the upper critical point of the ferrous metal base, raising the temperature of the surface metal of said workpiece to substantially 2000° F., maintaining said surface temperature for a time interval equivalent to substantially 15 minutes per inch thickness of said workpiece based on a highly luminous heat source, further raising the temperature of the surface metal to a selected working temperature between 2100 and 2400° F., maintaining the surface at said working temperature for a period of time substantially equal to 20 minutes per inch of thickness of said workpiece based on a highly luminous heat source, and work deforming the said heated workpiece to 35 form the desired worked article.

4. The method of manufacturing worked composite metal articles which comprises, heating a composite workpiece, made up of a carbon steel base to which is integrally united a chrome steel coating, to 1600° F., raising the temperature of the surface of said metal to 2000° F., maintaining said surface temperature for a period of time substantially equal to 15 minutes per inch of thickness of said workpiece based on a highly luminous flame, further raising the temperature of the surface metal to 2300° F., maintaining said surface temperature for a period of time substantially equal to 20 minutes per inch of thickness of said workpiece based on a highly luminous heat source, and work deforming the said heated workpiece to form the desired worked article.

ROBERT K. HOPKINS.